

## 1

3,114,697

**CATALYTIC REFORMING OF HYDROCARBONS**  
 Kenneth Hugh Bourne and Peter Thomas White, Sunbury-on-Thames, England, assignors to The British Petroleum Company Limited, London, England, a joint-stock corporation of Great Britain  
 No Drawing. Filed Aug. 18, 1959, Ser. No. 834,494  
 Claims priority, application Great Britain Aug. 27, 1958  
 2 Claims. (Cl. 208—136)

This invention relates to the dehydrogenation or dehydrocyclisation of non-aromatic hydrocarbons.

Catalysts of chromium oxide on a support, for example, alumina are known to have dehydrogenating and dehydrocyclising properties and various promoters have been proposed for improving such catalysts.

It has now been found that minor amounts of beryllium in combination with other promoters can improve supported chromium oxide catalysts and according to the present invention a process for the dehydrogenation or dehydrocyclisation of feedstocks consisting of or containing non-aromatic hydrocarbons comprises contacting the feedstock at a temperature of from 450 to 580° C. with a catalyst comprising chromium oxide on a support preferably alumina, the catalyst containing also a minor proportion (with respect to the chromium oxide) of beryllium and a minor proportion (with respect to chromium oxide) of an alkali metal, preferably potassium.

The beryllium and the alkali metal are preferably present in the form oxides. Preferably minor amounts, with respect to the chromium oxide, of one or more other promoting elements are present also, for example nickel, or cobalt. A catalyst containing minor amounts of beryllium, potassium and nickel is particularly preferred. The preferred proportions of catalyst components, by weight of total catalyst stable at 550° C., are:

|                                                               | Percent  |
|---------------------------------------------------------------|----------|
| Chromium oxide (expressed as Cr <sub>2</sub> O <sub>3</sub> ) | 5 to 25  |
| Beryllium (expressed as BeO)                                  | 0.1 to 5 |
| Potassium (expressed as K <sub>2</sub> O)                     | 0.1 to 5 |
| Other promoting elements (expressed as oxide)                 | 0.1 to 5 |
| Alumina                                                       | Balance  |

The process is preferably carried out at a pressure of not more than 50 p.s.i.g. without the addition of extraneous hydrogen and without recycle of the hydrogen-containing gas produced in the process. An appreciable quantity of such gas is produced, which is available as a valuable by-product. The term "not more than 50 p.s.i.g." includes atmospheric pressure or below, atmospheric pressure being in fact preferred. The preferred space velocity is 0.1 to 1.0 v./v./hr.

The catalyst may be used in the form of a fixed bed, a moving bed or a fluidised bed. Since it is readily regenerated by burning off carbonaceous deposits in a stream of oxygen-containing gas it is particularly suitable for fluidised or moving bed processes.

The feedstock used should boil within the gasoline or naphtha range (i.e. up to 200° C.) and may be pure hydrocarbons, for example straight chain paraffins or cycloparaffins, or mixtures of hydrocarbons. Preferably a major proportion of the feedstock boils below 100° C.

Thus according to one embodiment of the invention, the feedstock may be a straight-run gasoline fraction. By treatment according to the present invention gasolines or gasoline blending components having a research octane number (clear) of at least 90 may be obtained from such fractions. With feedstocks at the lower boiling end of the gasoline range the products will also have a high volatility and may be for example at least 50% volume evaporated at 100° C. A particularly preferred feedstock is a light gasoline having an end boiling point of about 80 to 120° C.

## 2

According to a further embodiment, the feedstock may be the product of a previous catalytic reforming process so that the present invention includes a two-stage reforming process designed to produce aromatics and high octane gasoline fractions with preferably a research octane number (clear) of the order of 100. Any convenient reforming process may be used as the first stage, but those employing a catalyst of platinum on a support containing aluminium oxide with or without halogen are preferred, such processes being hereinafter referred to as platinum reforming processes and the products as platinum reformates.

With a two-stage process, the whole of the reformate from the first stage may be reformed in the second stage. Alternatively the reformate may be fractionated and a portion only subjected to the further treatment. The portion may be a lower boiling relatively aromatic free fraction, preferably one with an end boiling point below 125° C. or a higher boiling fraction still containing some non-aromatic hydrocarbons. Alternatively the reformate may be solvent extracted and the raffinate or a fraction thereof subjected to the further treatment. If desired, the product may be recombined with the untreated fraction or the solvent extract as the case may be, but it may also be combined with other high octane components, for example heavy cat. cracked gasoline or alkylate.

The catalyst may be prepared by any convenient method.

Examples of suitable methods are:

(1) Impregnation of the alumina base with a solution containing the constituents, preferably in the form of salts. The base may be impregnated with all the constituents together, or two or more solutions containing different constituents may be used in succession. The impregnated base is dried and calcined.

(2) The alumina base may be co-precipitated from a solution, containing aluminium and either chromium or beryllium or both, with alkali, and the precipitate washed, dried, and calcined. The alkali metal may be subsequently added by impregnation, together with any constituent not co-precipitated. The catalyst is then again dried and calcined.

(3) An insoluble chromium or beryllium compound or both may be milled into the alumina base, further constituents added by impregnation and the catalyst dried and calcined.

(4) As for method 3 above except that the insoluble compound or compounds is suspended in a solution of an aluminium compound from which the alumina is precipitated.

The present invention includes a catalyst comprising chromium oxide on a support, preferably alumina, the catalyst containing also a minor proportion (with respect to the chromium oxide) of beryllium and a minor proportion (with respect to the chromium oxide) of an alkali metal, preferably potassium. The beryllium and the alkali metal are preferably present in the form of oxides. The catalyst may contain minor amounts of one or more other promoters as detailed above and the preferred proportions of catalyst components are also as set out above.

The invention is illustrated by the following examples:

## EXAMPLE 1

A solution containing 24 g. "Analal" chromium trioxide, 4 g. "Analal" potassium nitrate (KNO<sub>3</sub>), 5.5 g. beryllium nitrate [Be(NO<sub>3</sub>)<sub>2</sub>.3H<sub>2</sub>O] and 3 g. "Analal" nickel nitrate [Ni(NO<sub>3</sub>)<sub>2</sub>.6H<sub>2</sub>O] was used to impregnate 160 g. of alumina which had previously been calcined at 550° C. for two hours. The impregnated alumina was then dried for one hour at 130° C. and calcined for two hours at 550° C.

3  
EXAMPLE 2

A solution containing 24 g. "Analar" chromium trioxide, 4 g. "Analar" potassium nitrate ( $KNO_3$ ), 14 g. beryllium nitrate [ $Be(NO_3)_2 \cdot 3H_2O$ ], 3.5 g. "Analar" cobalt nitrate [ $Co(NO_3)_2 \cdot 6H_2O$ ] and 3.5 g. "Analar" nickel nitrate [ $Ni(NO_3)_2 \cdot 6H_2O$ ] was used to impregnate 160 g. of alumina which had previously been calcined at 550° C. for two hours. The impregnated alumina was then dried for one hour at 130° C. and calcined for two hours at 550° C.

4  
All figures are percentages by weight of total catalyst stable at 550° C.

The results are set out in Table 1 below.  
While catalyst 1 (promoted with beryllium and potassium) requires a higher temperature to reach a given octane number than some of the other catalysts, the yield obtained for any given octane number is good. Catalyst 2 (promoted with nickel and both beryllium and potassium) shows better results, particularly at the lower temperature, than either catalyst 3 or 4 (promoted with nickel and only one of either beryllium or potassium).

Table 1

| Reaction temperature----- |                                              | 475° C.                       |                              |                       |                              | 530° C.                         |                              |                         |                             |
|---------------------------|----------------------------------------------|-------------------------------|------------------------------|-----------------------|------------------------------|---------------------------------|------------------------------|-------------------------|-----------------------------|
|                           |                                              | Debutanised product           |                              | Exit gas              |                              | Debutanised product             |                              | Exit gas                |                             |
| Feed                      | Chromia/ alumina catalyst promoters          | Octane number research, clear | Yield, percent wt.           | Make, s.c.f./b.       | $H_2$ content, percent vol.  | Octane number research, clear   | Yield percent wt.            | Make, s.c.f./b.         | $H_2$ content, percent vol. |
| Light platinum reformate. | 1. Be-K<br>2. Ni-Be-K<br>3. Ni-K<br>4. Ni-Be | 89.8<br>98.8<br>96.3<br>84.5  | 96.9<br>88.5<br>87.5<br>81.8 | 517<br>1,100<br>1,379 | 86.8<br>89.0<br>89.0<br>89.0 | 100.0<br>103.8<br>104.8<br>96.7 | 82.5<br>69.5<br>68.0<br>60.1 | 1,345<br>1,889<br>2,305 | 83.3<br>79.0<br>78.0        |

## EXAMPLE 3

A solution containing 24 g. "Analar" chromium trioxide, 4 g. "Analar" potassium nitrate ( $KNO_3$ ) and 9 g. beryllium nitrate [ $Be(NO_3)_2 \cdot 3H_2O$ ] was used to impregnate 160 g. of alumina which had previously been calcined at 550° C. for two hours. The impregnated alumina was then dried for one hour at 130° C. and calcined for two hours at 550° C.

## EXAMPLE 4

A lower boiling fraction of a reformate obtained by hydroforming a naphtha fraction over a catalyst of platinum, alumina and combined halogen had an ASTM boiling range of 44° C.-110° C. and an octane number (research) clear of 80.0. This lower boiling fraction was

## EXAMPLE 5

30 Example 4 was repeated using a catalyst with the following composition:

|                                          | Percent wt. |
|------------------------------------------|-------------|
| Chromium oxide (expressed as $Cr_2O_3$ ) | 10          |
| Beryllium oxide (expressed as $BeO$ )    | 1.0         |
| Potassium oxide (expressed as $K_2O$ )   | 1.0         |
| Nickel oxide (expressed as $NiO$ )       | 0.5         |
| Cobalt oxide (expressed as $CoO$ )       | 0.5         |
| Alumina                                  | Balance     |

35 40 In addition comparative runs were carried out using a catalyst identical with the above except that it contained no beryllium.

The results are set out in Table 2 below.

Table 2

| Reaction temperature----- |                                     | 475° C.                       |                    |                 |                             | 530° C.                       |                   |                 |                             |
|---------------------------|-------------------------------------|-------------------------------|--------------------|-----------------|-----------------------------|-------------------------------|-------------------|-----------------|-----------------------------|
|                           |                                     | Debutanised product           |                    | Exit gas        |                             | Debutanised product           |                   | Exit gas        |                             |
| Feed                      | Chromia/ alumina catalyst promoters | Octane number research, clear | Yield, percent wt. | Make, s.c.f./b. | $H_2$ content, percent vol. | Octane number research, clear | Yield percent wt. | Make, s.c.f./b. | $H_2$ content, percent vol. |
| Light platinum reformate. | Co-Ni-Be-K<br>Co-Ni-K               | 96.9<br>97.3                  | 83.7<br>83.6       | 984<br>998      | 89.0<br>81.5                | 103.7<br>103.6                | 70.8<br>66.1      | 196.0<br>180.2  | 82.0<br>80.0                |

treated under the following process conditions:

Pressure ----- Atmospheric.  
Space velocity ----- 0.2 v./v./hr.  
Recycle gas ----- None.

Runs were carried out at two temperatures—475° C. and 530° C. Four catalysts were used as follows:

|                                          | 1       | 2       | 3       | 4       |
|------------------------------------------|---------|---------|---------|---------|
| Chromium oxide (expressed as $Cr_2O_3$ ) | 10      | 10      | 10      | 10      |
| Beryllium oxide (expressed as $BeO$ )    | 0.65    | 0.4     | 1.0     | 0.4     |
| Potassium oxide (expressed as $K_2O$ )   | 1.0     | 1.0     | 1.0     | 0.4     |
| Nickel oxide (expressed as $NiO$ )       |         |         | 0.4     | 0.4     |
| Alumina                                  | balance | balance | balance | balance |

The results show the improvement in yield obtained at the higher temperature by the addition of beryllium to the catalyst.

## EXAMPLE 6

65 A light gasoline having an ASTM boiling range of 41.5° C.-103° C. and an octane number (research) clear of 58.7 was treated under the following process conditions:

Pressure ----- Atmospheric,  
Space velocity ----- 0.2 v./v./hr.  
Recycle gas ----- None.  
Process period ----- 5 hours.

70 75 Runs were carried out at two temperatures—475° C. and 530° C.

Three catalysts were used as follows:

(i) A catalyst prepared as described in Example 1 and having the composition:

|                                                               | Percent wt. |
|---------------------------------------------------------------|-------------|
| Chromium oxide (expressed as Cr <sub>2</sub> O <sub>3</sub> ) | 10          |
| Beryllium oxide (expressed as BeO)                            | 0.4         |
| Nickel oxide (expressed as NiO)                               | 0.4         |
| Potassium oxide (expressed as K <sub>2</sub> O)               | 1.0         |
| Alumina                                                       | Balance     |

(ii) A catalyst similar with catalyst (i) but containing no potassium.

(iii) A catalyst similar with catalyst (i) but containing no beryllium.

Catalyst (ii) and (iii) were used for comparative purposes.

The results are set out in Table 3 below.

The results show that the catalyst containing both beryllium and potassium gave better results, particularly at the higher temperature than the other catalysts. At the higher temperature both yield and octane number were improved.

15

all percentages being by weight of total catalyst material stable at 550° C., at a temperature of 450 to 580° C., at a pressure not in excess of about 50 p.s.i. ga., at a space velocity of 0.1 to 1.0 v./v./hr., and in the absence of added hydrogen to the reaction zone, and recovering a product having an increased aromatic content.

2. A process for the treatment of a petroleum feedstock consisting essentially of non-aromatic hydrocarbons boiling within the range encompassed by the gasoline and naphtha range to produce a product having an increased aromatic content, comprising contacting the feedstock in a reaction zone with a catalyst consisting essentially of 5 to 25% of chromium oxide, expressed as Cr<sub>2</sub>O<sub>3</sub>; 0.1 to 5% of beryllium, expressed as BeO; 0.1 to 5% of an alkali metal, expressed as alkali metal oxide, about 0.1 to 5% of nickel, expressed as NiO; about 0.1 to 5% of cobalt, expressed as CoO, and balance alumina, all percentages being by weight of total catalyst material stable at 550° C., at a temperature of 450 to 580° C., at a pressure not in excess of about 50 p.s.i. ga., at a space velocity of 0.1 to 1.0 v./v./hr., and in the absence of

20

Table 3

| Feed               | Chromia/<br>alumina<br>catalyst<br>promoters | 475° C.                                |                          |                    |                                                | 530° C.                                |                          |                    |                                                |
|--------------------|----------------------------------------------|----------------------------------------|--------------------------|--------------------|------------------------------------------------|----------------------------------------|--------------------------|--------------------|------------------------------------------------|
|                    |                                              | Debutanised<br>product                 |                          | Exit gas           |                                                | Debutanised<br>product                 |                          | Exit gas           |                                                |
|                    |                                              | Octane<br>number<br>research,<br>clear | Yield,<br>percent<br>wt. | Make,<br>s.c.f./b. | H <sub>2</sub> con-<br>tent, per-<br>cent vol. | Octane<br>number<br>research,<br>clear | Yield,<br>percent<br>wt. | Make,<br>s.c.f./b. | H <sub>2</sub> con-<br>tent, per-<br>cent vol. |
| Light<br>gasoline. | [Ni-Be]<br>[Ni-Be-K]<br>[Ni-K]               | 84.5<br>82.1<br>82.5                   | 81.8<br>86.3<br>83.0     | 1879<br>1800       | 89.0<br>83.0                                   | 96.7<br>99.7<br>95.0                   | 60.1<br>63.5<br>60.0     | 2305<br>2461       | 78.0<br>79.5                                   |

We claim:

1. A process for the treatment of a petroleum feedstock consisting essentially of non-aromatic hydrocarbons boiling within the range encompassed by the gasoline and naphtha range to produce a product having an increased aromatic content, comprising contacting the feedstock in a reaction zone with a catalyst consisting essentially of 5 to 25% of chromium oxide, expressed as Cr<sub>2</sub>O<sub>3</sub>; 0.1 to 45

added hydrogen to the reaction zone, and recovering a product having an increased aromatic content.

#### References Cited in the file of this patent

##### UNITED STATES PATENTS

|           |                     |               |
|-----------|---------------------|---------------|
| 2,441,297 | Stirton             | May 11, 1948  |
| 2,705,733 | Nonnenmacher et al. | Apr. 5, 1955  |
| 2,754,345 | Kirshenbaum         | July 10, 1956 |
| 2,787,583 | McGrath et al.      | Apr. 2, 1957  |
| 2,897,135 | Doumani             | July 28, 1959 |
| 2,898,290 | Swabb               | Aug. 4, 1959  |